

## UNITED STATES PATENT OFFICE

1,932,862

## ALUMINUM ALLOYS

Robert T. Wood, Cleveland, Ohio, assignor to  
Aluminum Company of America, Pittsburgh,  
Pa., a corporation of Pennsylvania

No Drawing. Original application September 21,  
1932, Serial No. 634,155. Divided and this ap-  
plication November 30, 1932. Serial No.  
645,116

1 Claim. (Cl. 75—1)

This invention relates to aluminum base al-  
loys containing magnesium. The invention has  
for its object the improvement of alloys of this  
class by the addition thereto of about 0.05 to 2.0  
5 per cent by weight of calcium. The invention is  
particularly concerned with the specific alloys  
hereinafter described.

The claim of this application covers certain  
matter divided from my copending application  
10 Serial No. 634,155 which is, in part, a continuation  
of my copending application Serial No. 595,-  
231. Inventions disclosed but not claimed  
herein are claimed in my copending applica-  
tions Serial Nos. 595,231, filed February 25, 1932,  
15 645,108 to 645,115 inclusive, and 645,117 to 645,-  
125 inclusive, all filed November 30, 1932.

Considerable difficulty has heretofore been en-  
countered in attempts to commercially produce  
20 castings of aluminum base alloys containing sub-  
stantial amounts of magnesium. This difficulty  
is encountered both in the making of sand cast-  
ings and permanent mold or chill-mold cast-  
ings, although the nature of the difficulty dif-  
fers somewhat in each case. In the case of sand  
25 castings there occurs a reaction between the  
molten aluminum base alloy containing mag-  
nesium and the ordinary sand-mold materials,  
or vapors generated therefrom. There is also a  
reaction with the atmosphere. In addition, the  
30 magnesium-containing aluminum base alloy  
does not flow freely through narrow mold sec-  
tions at ordinary pouring temperatures and, if  
the pouring temperature be raised, the solidified  
alloy is unsound. If the aluminum base alloy  
35 containing magnesium be cast in a chill-mold  
the reaction effect is minimized to some extent,  
but the troubles arising from cold-shuts and  
mis-runs are accentuated because of the more  
rapid chilling of the molten metal. The con-  
40 siderations apply to the aluminum base alloys  
specifically disclosed herein and particularly to  
such alloys.

I have discovered that when calcium is added  
45 to aluminum base alloys of the type and com-  
position herein described, these difficulties are,  
to a considerable extent, eliminated. The cal-  
cium should be present in amounts ranging from  
0.05 per cent to 2.0 per cent by weight subject to  
50 specific considerations as hereinafter disclosed.

positions herein described, a viscous scum often  
forms at the surface of the molten metal. Fail-  
ure of the molten metal to run properly through  
narrow mold apertures is caused, in part, by  
shreds or particles of this scum being suspended  
35 in the molten metal and offering a resistance to  
the free passage of the metal through the aper-  
tures. Regardless of the cause of this low fluidi-  
ty, I have discovered that the addition to the  
alloy of relatively small amounts of calcium,  
40 in the preferred range between 0.05 to 0.5 per  
cent, improves the casting characteristics to a  
very considerable extent and simultaneously ef-  
fects a reduction of the scum or dross collecting  
at or near the surface. In the casting of arti-  
55 cles in sand molds, I prefer to add calcium in  
amounts less than about 0.5 per cent except in  
instances where some reduction of tensile  
strength or other mechanical or tensile prop-  
erty is immaterial. In amounts of more than  
60 0.5 per cent the calcium addition produces the  
advantages enumerated herein but has a tend-  
ency to lower some of the physical properties  
of the alloys. This effect is not harmful when  
70 calcium is present in amounts of about 0.5 per  
cent or less, but when high strength is not a  
desideratum the calcium may be used in  
amounts up to about 2.0 per cent. In intricate  
75 permanent mold castings, where casting troubles  
are very serious if no calcium be added, the im-  
proved physical properties obtained coincident  
80 with the production of good castings more than  
offset the diminution in properties which might  
otherwise result from the use of the calcium.

I have also discovered that when calcium is  
85 added to aluminum base alloys containing mag-  
nesium, the amount of gas evolved during solidi-  
fication of the alloys is considerably reduced.  
When from about 0.05 per cent to 2.0 per cent  
by weight of calcium is added to the alloys, the  
90 amount of gas evolved becomes less marked with  
increasing calcium content and the reduction of  
gas evolution may be so marked that the molten  
metal cools to the solidification temperature with  
a smooth mirror-like surface. I prefer to re-  
95 strict the amount of calcium added to 2.0 per  
cent or less since above this amount the physi-  
cal properties of the alloys may be too seriously  
affected. If the best physical properties are de-  
sired with an improved, although not complete,  
100

degree of gas prevention, I keep the calcium content of the alloys between 0.05 per cent and about 0.5 per cent.

In the application of the principles of my invention I have determined that certain aluminum base alloys containing magnesium are particularly benefited thereby. For example, a very useful aluminum base alloy is one containing about 2.0 to 9.0 per cent of magnesium and 0.05 to 10 per cent to 2.0 per cent of calcium, as is also aluminum base alloy containing about 2.0 to 15.0 per cent of magnesium, 0.1 to 3.5 per cent of cobalt, and 0.05 to 2.0 per cent of calcium to which other elements such as copper, antimony, bismuth, nickel, manganese, and other well known alloying elements may be added to produce particular properties therein.

Likewise is the addition of 0.05 to 2.0 per cent of calcium beneficial to those aluminum base alloys which contain about 2.0 to 15.0 per cent of magnesium and 0.05 to 0.4 per cent of at least one of the class of metals here defined as antimony and bismuth, such alloys being very useful where use at high temperatures is contemplated. Calcium may likewise be added to improve such alloys when they contain, in addition to magnesium and antimony and/or bismuth, one or more of such alloying elements as cobalt, copper, nickel, manganese, zinc, etc. which may be added to modify or produce a specific property in the alloy.

The addition of 0.05 to 2.0 per cent of calcium is very beneficial in the case of a series of aluminum base alloys which contain as major alloying elements about 2.0 to 10.0 per cent of magnesium and about 0.2 to 5.0 per cent of nickel. For instance, an aluminum base alloy containing 3.0 to 7.5 per cent of magnesium and 0.2 to 2.0 per cent of nickel is improved by the addition of 0.05 to 2.0 per cent of calcium as is, likewise, this same alloy when it also contains about 0.05 to 0.4 per cent of one or more of the class of elements composed of antimony and bismuth. Another excellent aluminum base alloy prepared in accordance with the principles of my invention is one containing 3.0 to 8.0 per cent of magnesium, 0.5 to 4.0 per cent of nickel, 0.5 to 4.0 per cent of manganese, and 0.05 to 2.0 per cent of calcium, which alloy may also be improved, particularly for application at high temperatures, by the addition of 0.05 to 0.4 per cent of at least one of the class of elements composed of antimony and bismuth.

The principles of my invention find particular application in the case of aluminum base alloys containing magnesium, nickel, and chromium, and aluminum base alloys containing magnesium, nickel, and copper, as well as those alloys containing magnesium, nickel, and cobalt. Examples may be given of aluminum base alloys containing 2.0 to 10.0 per cent of magnesium, 0.2 to 5.0 per cent of nickel, 0.5 to 3.5 per cent of chromium, and 0.05 to 2.0 per cent of calcium. An aluminum base alloy containing 3.0 to 8.0 per cent of magnesium, 0.5 to 3.5 per cent of nickel, 0.5 to 3.5 per cent of chromium, and 0.05 to 0.4 per cent of cobalt.

to 2.0 per cent of calcium has excellent casting properties and the high temperature properties of this alloy can be favorably affected by the addition of 0.05 to 0.4 per cent of at least one of a class of elements composed of bismuth and antimony. Examples may be given of aluminum base alloy containing 2.0 to 10.0 per cent of magnesium, 0.2 to 5.0 per cent of nickel, 1.0 to 6.0 per cent of copper, and 0.05 to 2.0 per cent of calcium. An excellent alloy of this type is one containing 3.0 to 8.0 per cent of magnesium, 0.5 to 5.0 per cent of nickel, 1.0 to 6.0 per cent of copper, and 0.05 to 2.0 per cent of calcium with or without 0.05 to 0.4 per cent of at least one of the class of elements composed of antimony and bismuth and with or without the further addition of 0.5 to 3.5 per cent of at least one of a class of elements composed of cobalt and chromium, and with or without the further addition of 0.1 to 1.0 per cent of at least one of a class of elements composed of tungsten, vanadium, molybdenum, titanium, and zirconium.

Other excellent alloys are those aluminum base alloys containing about 2.0 to 10.0 per cent of magnesium, 0.2 to 5.0 per cent of nickel, 0.1 to 3.5 per cent of cobalt, and 0.05 to 2.0 per cent of calcium. A particular example of this class of alloys, which may also contain with considerable advantage 0.05 to 0.4 per cent of a class of elements composed of antimony and bismuth, is the aluminum base alloy containing 3.0 to 8.0 per cent of magnesium, 0.5 to 4.0 per cent of nickel, 0.1 to 3.0 per cent of cobalt, and 0.05 to 2.0 per cent of calcium.

Among other magnesium-containing aluminum base alloys which I have found to be particularly benefited by the presence of calcium are numbered the aluminum base alloys containing 3.0 to 8.0 per cent of magnesium, 1.0 to 6.0 per cent of copper, 0.5 to 3.5 per cent of chromium, and 0.05 to 2.0 per cent of calcium, with or without the addition of 0.05 to 0.4 per cent of at least one of a class of metals composed of antimony and bismuth and with or without the addition of other alloying elements.

The alloys herein described may be produced by the usual methods of alloying metals. The calcium is preferably added to the molten alloy by thrusting the calcium beneath the surface with tongs or other suitable instrument. The aluminum used in preparing the alloys may be pure or it may contain the impurities found in commercial grades of this metal. Ordinarily a good commercial grade of virgin aluminum will give excellent results and is preferable.

Having thus explained and described my invention, I claim:

A metallic alloy consisting of 3.0 to 8.0 per cent by weight of magnesium, 0.5 to 5.0 per cent by weight of nickel, 1.0 to 6.0 per cent by weight of copper, 0.05 to 0.4 per cent by weight of at least one of a class of elements composed of antimony and bismuth, and 0.05 to 2.0 per cent by weight of calcium, the balance being aluminum.

ROBERT T. WOOD. 145